

## STABLE PETROLEUM DISTILLATE FUELS

Kurt F. Richards, Dyer, Ind., assignor to Standard Oil Company, Chicago, Ill., a corporation of Indiana

No Drawing. Application November 30, 1953  
Serial No. 395,271

14 Claims. (Cl. 44—66)

This invention relates to stable petroleum oils and it is particularly concerned with the stabilization of hydrocarbon oils normally susceptible to oxidative deterioration at normal storage temperatures.

The deterioration of petroleum fractions, e.g. in the distillate oil range, manifests itself through the appearance of color, sediment, etc. in the oil. Sediment formation is particularly troublesome in oils used as fuel's because it often results in clogging of equipment such as filters, screens, and nozzles. Petroleum fractions generally, however, with the possible exception of highly refined lubricating oils, are subject to oxidative deterioration in storage. And the prevention of such deterioration along with provision for finely dispersing and insoluble matter present in an oil are problems of extreme importance to the refiner.

It is an object of the present invention to provide an additive for petroleum oils which will inhibit sedimentation, color formation, etc. and other undesirable deterioration. It is another object to disperse, and to thus render harmless, any sludge or color deterioration products occurring in such oils. Still another object is to provide a fuel oil resistant to sediment formation and sludging.

It is a further object of the present invention to provide sludge-preventing additives for fuel oils comprising mixtures of virgin distillate and a cracked oil in the distillate fuel boiling range. These and additional objects will be apparent from the following detailed description of the present invention.

In accordance with the present invention, sediment formation may be prevented and oils of good color and overall stability may be assured by adding to petroleum oils a small amount of at least one polyamino compound of the hereinafter defined class along with a neutralized reaction product of a phosphorus sulfide and a hydrocarbon. More specifically, it has been found that a high degree of stabilization of petroleum fractions normally subject to oxidative deterioration upon storage at normal temperatures may be obtained by adding thereto a small amount of a neutralized reaction product of a phosphorus sulfide and a hydrocarbon, e.g. that of  $P_2S_5$  and a butylene polymer, and at least one N-alkyl-propylene diamine compound (containing from about 6 to about 30 carbon atoms as the N-alkyl radical) selected from the group consisting of N-alkyl alkylene polyamines containing one primary amino nitrogen atom and carboxylic acid salts thereof. These constituents are added in amounts sufficient to inhibit deterioration, e.g. generally from about 0.001% to about 0.1% and preferably from about 0.005 to about 0.05%. Thus, for example, distillate fuel oils containing about 0.005% of an additive comprising 0.004% of an N-alkyl propylene diamine, 0.001% of an oleic acid salt of such amine, and 0.005% of a neutralized reaction product of  $P_2S_5$  and butylene polymer have shown striking stability as compared to the same oils without such additive. Not only has such additive shown

an outstanding ability to stabilize such oils from deterioration resulting in discoloration, sediment, etc., but in addition to be able to disperse any sediment which might form or which might have been present in the oil prior to introducing the additive and to impart substantial corrosion inhibiting properties to the oil.

More specifically, there may be employed such amines as N-n-cetyl-propylene diamine, the various "Duomeens" (products of Armour Chemical Division) which have the general formula  $RNHCH_2CH_2CH_2NH_2$  wherein R may be derived from coconut fatty acid ("Duomeen C"), from tallow fatty acid ("Duomeen T"), from lauric acid ("Duomeen 12"), or from soya fatty acid ("Duomeen S"), etc. The "Duomeens" are industrial or technical grade chemicals with an amine content of approximately 80% calculated as diamine. The approximate melting ranges for each of the aforementioned "Duomeens" are: "Duomeen C"—20° to 24° C., "Duomeen 12"—28 to 32° C., "Duomeen S"—38° to 42° C., and "Duomeen T"—44° to 48° C.

Phosphorus sulfide-hydrocarbon reaction products of the type which may be employed in accordance herewith may be readily obtained by reacting a phosphorus sulfide with a hydrocarbon at a temperature of from about 200° F. to about 600° F., and preferably from about 250° F. to about 500° F., using from about 1% to about 50%, and preferably from about 5% to about 25%, by weight, of the phosphorus sulfide in the reaction. It is advantageous to maintain a non-oxidizing atmosphere, such as for example, an atmosphere of nitrogen above the reaction mixture. Usually, it is preferable to use an amount of the phosphorus sulfide that will completely react with the hydrocarbon so that no further purification becomes necessary; however, an excess of phosphorus sulfide can be used and separated from the product by filtration or by dilution with a solvent, such as hexane, filtering and subsequently removing the solvent by suitable means, such as by distillation. The phosphorus sulfide-hydrocarbon reaction products contain both sulfur and phosphorus. The reaction may if desired be carried out in the presence of an additional sulfurizing agent or the phosphorus sulfide-hydrocarbon reaction product can be sulfurized, as described in U.S. 2,316,087 issued April 6, 1943, to James W. Gaynor and Clarence M. Loane.

The hydrocarbon constituent of this reaction is preferably a mono-olefin hydrocarbon polymer resulting from the polymerization of low molecular weight mono-olefinic hydrocarbons or isomono-olefinic hydrocarbons, such as propylene, butylenes, and amylanes or the copolymers obtained by the polymerization of hydrocarbon mixtures containing isomono-olefins and mono-olefins or mixtures of olefins in the presence of a catalyst, such as sulfuric acid, phosphoric acid, boron fluoride, aluminum chloride or other similar halide catalysts of the Friedel-Crafts type.

The polymers employed are preferably mono-olefin polymers or mixtures of mono-olefin polymers and iso-mono-olefin polymers having molecular weights ranging from about 150 to about 50,000 or more, and preferably from about 300 to about 10,000. Such polymers can be obtained, for example, by the polymerization in the liquid phase of a hydrocarbon mixture containing mono-olefins and isomono-olefins such as butylene and isobutylene at a temperature of from about —80° F. to about 100° F. in the presence of a metal halide catalyst of the Friedel-Crafts types such as, for example, boron fluoride, aluminum chloride, and the like. In the preparation of these polymers there may be employed, for example, a hydrocarbon mixture containing isobutylene, butylenes and butanes recovered from petroleum gases, especially those gases produced in the cracking of petroleum oils in

the manufacture of gasoline. U.S. 2,407,873 to Evening et al. describes a particularly suitable technique for polymerizing such olefins in the presence of an aluminum-chloride-hydrocarbon complex catalyst.

Essentially paraffinic hydrocarbons such as bright stock residuums, lubricating oil distillates, petrolatums or paraffin waxes may be used. The condensation products of any of the foregoing hydrocarbons or their halogen derivatives, with aromatic hydrocarbons can also be employed.

Examples of high molecular weight olefinic hydrocarbons which can be employed as reactants are cetene ( $C_{16}$ ), cerotene ( $C_{26}$ ), melene ( $C_{30}$ ), and mixed high molecular weight alkenes obtained by cracking petroleum oils. Other olefins suitable for the preparation of the herein described phosphorus sulfide reaction products are olefins having at least 20 carbon atoms in the molecule of which from about 12 carbon atoms to about 18 carbon atoms, and preferably at least 15 carbon atoms, are in a long chain. Such olefins can be obtained by the dehydrogenation of paraffins, such as by the cracking of paraffin waxes, or by the dehalogenation of alkyl halides, preferably long chain alkyl halides, particularly halogenated paraffin waxes. Also, olefins derived from the synthol or hydrocarbon syntheses process may be employed. These are essentially straight chain compounds varying widely in molecular weight.

Also contemplated within the scope of the present invention are the reaction products of a phosphorus sulfide with aromatic hydrocarbons such as benzene, naphthalene, anthracene, toluene, diphenyl, etc. and alkylated aromatic hydrocarbon such as, for example, an alkyl benzene characterized by having at least one alkyl group of at least four carbon atoms, and preferably at least eight carbon atoms such as a long chain paraffin wax.

The phosphorus sulfide reactant can be any phosphorus sulfide, such as for example,  $P_2S_3$ ,  $P_4S_3$ ,  $P_4S_7$ , and preferably  $P_2S_5$ .

The phosphorus sulfide-hydrocarbon reaction product normally shows a titratable acidity which is neutralized by treatment with a basic reagent. The phosphorus-sulfide-hydrocarbon reaction product when neutralized with a basic reagent containing a metal constituent is characterized by the presence or retention of the metal constituent of the basic reagent. Other metal constituents such as a heavy metal constituent can be introduced into the neutralized product by reacting the same with a salt of the desired heavy metal.

The term "neutralized phosphorus sulfide-hydrocarbon reaction product" as used herein means a phosphorus sulfide hydrocarbon reaction product having at least about 1% of its titratable acidity neutralized by the reaction with a basic reagent and includes the neutralized phosphorus sulfide-hydrocarbon reaction products containing a metal constituent resulting from said neutralization or resulting from the double decomposition of the phosphorus sulfide-hydrocarbon reaction product treated with a heavy metal salt.

The neutralized phosphorus sulfide-hydrocarbon reaction product can be obtained by treating the reaction product with a suitable basic compound such as a hydroxide, carbonate, sulfide, or an oxide of an alkaline earth metal, e.g. calcium or barium, and preferably the latter, or an alkali metal such as, for example, potassium hydroxide or sodium hydroxide. Other basic reagents can be used such as, for example, ammonia or an alkyl or aryl substitute of ammonia such as amines. The products are neutralized by mixing a suitable base (e.g. a 50% solution of KOH) therewith and heating to a temperature in the range of from about 200° to about 400° F. After the base and phosphorus sulfide hydrocarbon reaction product are mixed and neutralized, they are preferably steamed at a temperature of about 400° F. to about a half hour. The steaming may take place during neutralization.

For a more complete description of neutralized products of this type and method of obtaining same, reference is made to U.S. 2,316,080, 2,316,082 and 2,377,955.

The salts of the polyamines which may be employed in accordance herewith may be prepared by reacting, under carefully controlled, non-dehydrating conditions, i.e. below about 200° F. and preferably below about 195° F., a carboxylic acid containing from about 6 to about 20 carbon atoms, and preferably at least about 12 carbon atoms, e.g. hexanoic, nonanoic, lauric, stearic, oleic, linoleic, linolenic, palmitic, etc., with any of the hereinabove described amines to obtain either the mono- or di-substituted acid salts of the amines. Care must be taken in the preparation of such salts inasmuch as prolonged exposure to temperatures higher than about 200° F. results in the formation of amides or even glyoxalidines (if 1,2-substituted polyamines are employed) upon splitting out water. Among the very economical, commercially available salts of this type are the oleic acid mono- and/or di-salts of the Duomen (above described), particularly of Duomeen T.

Whereas the additive of the present invention is generally useful in petroleum distillates, and particularly cracked distillate fuels, it is especially useful in stocks of the type generally referred to as light catalytic cycle oil and fuel containing such an oil. Such a catalytic cycle oil is obtained from a catalytic hydrocarbon cracking operation in which a gas oil or heavier hydrocarbons such as reduced crude is cracked at a temperature of about 800° F. to about 1050° F. at a pressure of about atmospheric to about 50 pounds per square inch in the presence of suitable catalysts, such as for example silica-magnesia, silica-alumina, and other well-known cracking catalysts. A method of conducting a fluidized catalytic cracking operation is described in U.S. 2,341,193 issued to Fred W. Scheineman, February 8, 1944. The product fraction referred to herein is the heavier-than-gasoline fraction ordinarily called light gas oil or catalytic light cycle stock. A catalytic light cycle stock of the type particularly suitable for blending with virgin heavy distillates is a fraction having an aromatic content of at least about 40 to about 50% and a distillation range between about 425° F. and about 560° F. A typical analysis of a suitable light catalytic cycle stock shows the material to be composed substantially of about 10% normal  $C_{12}$  paraffins, about 45% of other paraffins and naphthenes, about 5% mono-nuclear aromatics which are mainly mono- to hexa-alkylated benzenes, and about 40% polynuclear aromatics which are mainly alkyl naphthalenes, largely methylated naphthalenes. The boiling range of a typical light catalytic cycle stock by A.S.T.M. distillation may be approximately:

|                       | ° F. |
|-----------------------|------|
| Initial boiling point | 430  |
| 10% over              | 448  |
| 50% over              | 478  |
| 90% over              | 518  |
| Maximum boiling point | 552  |

The boiling range of particular cycle oils may, of course, vary over a considerably wider range, depending upon catalyst, cracking conditions, charge stock, etc. Thus, catalytic cycle oils, generally, may boil within the range from about 350° F. to about 750° F.

It should be understood that the additives of this invention will inhibit oxidative deterioration in normally liquid petroleum fractions which are subject to the same under normal storage conditions. Such fractions may be cracked (thermally or catalytically) or virgin or mixtures of these. Thus, petroleum distillates generally such as internal combustion engine fuels, furnace oils, burner oils, heater oils, kerosene, heavy industrial residual fuels (e.g. Bunker C), jet fuels, blending oils, stripper stocks, etc.,

may be stabilized in accordance herewith. The oils to which the additives of the present invention are added may have been refined by any of the many well-known techniques, e.g. caustic washing, acid treatment, Doctor sweetening, clay treating, etc., prior to additive introduction.

The oils which may be stabilized by the additives of the present invention may be cracked, virgin or mixtures of these. Even blends of two different virgin oils, which

an oleic acid salt of Duomeen T demonstrated the effectiveness of such combination to be about the equal of the polyamine plus the neutralized phosphorus and sulfur containing compound. Whereas, a two-component additive, i.e. polyamine or polyamine oleate plus neutralized  $P_2S_5$  butylene polymer, gives excellent protection, the combination of polyamine, polyamine salt and neutralized phosphorus sulfide-hydrocarbon reaction product gives a substantially improved result.

Table 1

|                                       | No Additive                 | KOH-Neutralized $P_2S_5$ -butylene polymer (ca. 1,000 mol. wt.) product <sup>1</sup> plus A <sup>2</sup> | Neutralized $P_2S_5$ -butylene (ca. 1,000 mol. wt.) product <sup>1</sup> plus A <sup>2</sup> +B <sup>3</sup> |
|---------------------------------------|-----------------------------|----------------------------------------------------------------------------------------------------------|--------------------------------------------------------------------------------------------------------------|
| Rust protection: <sup>4</sup>         |                             |                                                                                                          |                                                                                                              |
| (1) Water layer—                      |                             |                                                                                                          |                                                                                                              |
| 24 hours.....                         | Severe rust.....            | No rust.....                                                                                             | No rust.....                                                                                                 |
| 144 hours.....                        | do.....                     | do.....                                                                                                  | Do.....                                                                                                      |
| 300 hours.....                        | do.....                     | Rust on edges.....                                                                                       | Do.....                                                                                                      |
| (2) Oil layer—                        |                             |                                                                                                          |                                                                                                              |
| 24 hours.....                         | do.....                     | No rust.....                                                                                             | Do.....                                                                                                      |
| 144 hours.....                        | do.....                     | do.....                                                                                                  | Do.....                                                                                                      |
| 300 hours.....                        | do.....                     | do.....                                                                                                  | Do.....                                                                                                      |
| Filterability <sup>5</sup> after—     |                             |                                                                                                          |                                                                                                              |
| 50 ml.....                            | 110 seconds.....            | 26 seconds.....                                                                                          | 22 seconds. <sup>6</sup>                                                                                     |
| 200 ml.....                           | 335 seconds.....            | 30 seconds.....                                                                                          | 24 seconds. <sup>6</sup>                                                                                     |
| 400 ml.....                           |                             | 34 seconds.....                                                                                          | 26 seconds. <sup>6</sup>                                                                                     |
| Crucible mat <sup>7</sup> —           | Many brown-gray specks..... | Brown tint and specks.....                                                                               | Few small gray specks.....                                                                                   |
| Appearance after aging <sup>7</sup> — | Cloudy.....                 | Slightly cloudy.....                                                                                     | Bright.....                                                                                                  |
| Color after aging <sup>7</sup> —      | Dark.....                   | Light.....                                                                                               | Light.....                                                                                                   |
| Sediment after aging <sup>7</sup> —   | Very much.....              | Trace.....                                                                                               | None.....                                                                                                    |

<sup>1</sup> Employed in amount of 0.005%.

<sup>2</sup> A=Duomeen T (Armour Chemical Division)—employed in an amount of 0.005%.

<sup>3</sup> B=Duomeen T Oleate (Armour Chemical Division)—employed in amount of 0.001%.

<sup>4</sup> 50 milliliter samples of furnace oil were filtered into bottles and doped with additive. Bright steel strips were immersed in the oil for 5 minutes, then withdrawn. Twenty-five milliliters of water were added to the bottles, and the bottles were thoroughly shaken. The steel strips were then reimmersed and left to stand in the open bottles for 144 hours. The strips were then withdrawn, dipped in mineral oil, allowed to drain, and hung in room air. The strips were examined after 24, after 144, and after 300 hours.

<sup>5</sup> 500 milliliter samples of furnace oil, with and without additive, were aged in open bottles in an oven for 20 hours at about 220° F. The samples were allowed to cool, and then filtered through 1 square centimeter of filter paper having a pore size of 10 microns, using a constant head of 12 inches of oil. The time necessary to collect successive 50 ml. increments of oil was recorded. The time required for the first, fourth and eighth 50 ml. portions is given above. The high sediment and gum content oil becomes progressively harder to filter whereas the time for those containing the additive changes very little from start to finish.

<sup>6</sup> 500 milliliter samples of furnace oil, with and without additive, were shaken with 500 ml. of tap water in a separatory funnel. The oil and water layers were allowed to separate for 30 minutes; the free water was then drawn off, and the interfacial rag and the oil layer were filtered through a medium porosity fritted-glass crucible. The color and nature of the mat retained in the crucible indicate the tendency of the oil to sludge after contact with water. The lighter the mat the less the sludging tendency.

<sup>7</sup> At the completion of the filtration, data for which are set forth above under "Filterability," the filtered samples were returned to bottles and stoppered and then allowed to stand at room temperature for seven days. The results given are a result of visual examination.

<sup>8</sup> Run with different sample of control oil but under essentially identical conditions.

because of solubility differences result in the formation of sediment when admixed, may be stabilized thereby.

The herein described additives are outstanding in many ways. Thus, the additive imparts rust protection to metal surfaces in contact with the oil, inhibits sediment formation, improves filterability by dispersing any sediment formed, inhibits color degradation, decreases wear of internal combustion engine parts (as demonstrated by the data in Table 3), etc. In Table 1, therefore, laboratory data are set forth which serve to demonstrate many of these improvements. The footnotes (1 through 4) to Table 1 explain the tests employed and their significance. Field tests have borne out the expected superiority of the additive in commercial use. Many gallons of potentially sediment-containing fuel oil have been successfully inhibited against this and other results of deterioration by the use of the additive of the present invention in actual commercial shipments. Filters which were on the verge of clogging when the use of oil containing such an additive was begun were found to have been substantially de-coated and unclogged after using the inhibited oil for several months. In those tests where new, clean filters were installed at the outset of the test they were like new several months later whereas other new filters installed at the same time in systems employing uninhibited oil were heavily coated and subject to clogging at any moment.

Additional tests of the type set forth in Table 1 on the same type fuel oil inhibited with a small amount of a neutralized  $P_2S_5$ -butylene polymer reaction product and

Accordingly, it should be understood that whereas either of such two component additives will give excellent results in accordance herewith it is preferred to employ all three, i.e. polyamine, polyamine-carboxylic acid salt and neutralized phosphorus sulfide-hydrocarbon reaction product. Of the two component additives, it is preferred to employ that comprising the polyamine rather than salt thereof.

In Table 2 are set forth data demonstrating the effectiveness of a rather wide variety of amines and phosphorus-sulfide hydrocarbon reaction products. These data are of a qualitative nature and clearly demonstrate on a laboratory scale the ability of the additives of the present invention to inhibit color degradation, sediment formation, etc. in a furnace oil comprising 60% virgin distillate and 40% fresh, caustic washed catalytic cycle oil. Data are included which compare the effectiveness of the herein disclosed polyamines with other amines which have heretofore been added to petroleum oils for various purposes. The data in Table 2 with the exception of the appearance of the crucible mat are based on the appearance of a furnace oil having the same composition as that employed in the tests recorded in Table 1, containing the additives indicated, after being heated for 20 hours at 200° F. and then held at room temperature for an additional 48 hours. The crucible data are obtained on the same oils in accordance with the test described in footnote 3 of Table 1, prior to heating the oils for 20 hours at 200° F.

Table 2

| Example     | Amine                              |        | P <sub>2</sub> S <sub>5</sub> -Butylene Polymer (ca. 1,000 mol. wt.) Reaction Prod. |        | "Duomeen T Oleate" | Appearance of Crucible After Test <sup>1</sup> | Color | Brightness | Sediment  |
|-------------|------------------------------------|--------|-------------------------------------------------------------------------------------|--------|--------------------|------------------------------------------------|-------|------------|-----------|
|             |                                    | Amount |                                                                                     | Amount |                    |                                                |       |            |           |
| 1 (control) | Duomeen T                          | .004   | A <sup>2</sup>                                                                      | .005   | .001               | Deep purple flecks                             | Dark  | V. cloudy  | Much.     |
| 2           | do                                 | .005   | B <sup>3</sup>                                                                      | .095   | do                 | Light pink cast                                | Light | Clear      | None.     |
| 3           | Duomeen C                          | .004   | A                                                                                   | .005   | do                 | Gray cast                                      | do    | do         | Do.       |
| 4           | Duomeen T                          | .004   | B                                                                                   | .005   | do                 | do                                             | do    | Sl. cloudy | Do.       |
| 5           | Duomeen S                          | .004   | A                                                                                   | .005   | do                 | do                                             | do    | V. clear   | Do.       |
| 6           | Duomeen 12                         | .004   | A                                                                                   | .005   | do                 | Gray brown cast                                | do    | Clear      | Do.       |
| 7           | N-n-dodecylethylene-diamine        | .004   | A                                                                                   | .005   | do                 | Deep gray cast                                 | do    | do         | Do.       |
| 8           | N-n-lauryldiethylene-diamine       | .004   | A                                                                                   | .005   | do                 | Pink cast                                      | do    | Cloudy     | Moderate. |
| 9           | Duomeen T                          | .004   | A                                                                                   | .005   | do                 | do                                             | do    | Sl. cloudy | Trace.    |
| 10          | Phenylenediamine                   | .005   | A                                                                                   | .005   | do                 | do                                             | do    | V. clear   | None.     |
| 11          | N-hydroxy dodecylethylene-triamine | .004   | A                                                                                   | .005   | do                 | Chocolate mat                                  | Dark  | Cloudy     | Much.     |
| 12          |                                    |        |                                                                                     |        | do                 | Tan gray cast                                  | Light | Sl. cloudy | Trace.    |

<sup>1</sup> See footnote 6 to Table 1 (supra) for explanation of test resulting in these observations.<sup>2</sup> A = KOH neutralized and steamed (at 400° F.) reaction product of P<sub>2</sub>S<sub>5</sub> and butylene polymer.<sup>3</sup> B = Ba(OH)<sub>2</sub> neutralized and steamed (at 400° F.) reaction product of P<sub>2</sub>S<sub>5</sub> and butylene polymer.

The surprising ability of additives of the present invention in preventing wear of internal combustion engine parts is demonstrated in Table 3. A diesel fuel comprising 60% straight run and 40% catalytic cycle oil having 0.1% concentration of an additive comprising 40% Duomeen T, 10% Duomeen T-mono-oleate and 50% of a potassium hydroxide neutralized reaction product of P<sub>2</sub>S<sub>5</sub> and a butylene polymer having a molecular weight of about 1000, was compared with the same oil without the additive in a General Motors 1-17 Diesel engine. This engine is a typical one-cylinder model of the General Motors "71" series engines.

Table 3

|                           | Control (Undoped Diesel Fuel) | Diesel Fuel Plus Additive |
|---------------------------|-------------------------------|---------------------------|
| Top compression ring:     |                               |                           |
| (a) Weight loss (grams)   | 0.91                          | 0.29                      |
| (b) Gap increase (inches) | 0.032                         | 0.006                     |
| Total compression rings:  |                               |                           |
| (a) Weight loss (grams)   | 2.03                          | 0.38                      |
| (b) Gap increase (inches) | 0.078                         | 0.013                     |

Other tests in which a diesel fuel comprising 100% of a low sulfur catalytic cycle oil was employed in the same engine, the improvement resulting from the presence of 0.1% of the additive was about 80% reduction of top ring wear and about 90% of total compression ring wear. Additional tests in a Caterpillar one cylinder test diesel engine demonstrated much the same improvement in wear characteristics.

As indicated above, the additives of the present invention are useful in straight run stocks (virgin) and blends of different virgin stocks. Thus, as shown in Table 4, the improved color inhibition in such oils when employing an additive of the present invention is substantial.

Table 4

| Oil                                           | Color (Saybolt) |                   |
|-----------------------------------------------|-----------------|-------------------|
|                                               | Initial         | Aged <sup>4</sup> |
| Control (A) <sup>1</sup>                      | +13             | -2                |
| Control (A) +0.01% of Additive <sup>2</sup>   | +13             | +10               |
| Control (A) +0.0025% of Additive <sup>2</sup> | +13             | +10               |
| Control (A) +0.001% of Additive <sup>2</sup>  | +13             | +8                |
| Control (B) <sup>3</sup>                      | +13             | -6                |
| Control (B) +0.0025% of Additive <sup>2</sup> | +13             | +5                |

<sup>1</sup> Blend of CuCl<sub>2</sub> sweetened Mid-Continent virgin heater oil distillate and sulfuric acid treated West Texas virgin heater oil distillate.<sup>2</sup> 50% KOH neutralized reaction product of P<sub>2</sub>S<sub>5</sub> and butylene polymer of about 1000 molecular weight, 40% of Duomeen T and 10% of Duomeen T mono-oleate.<sup>3</sup> Sulfuric acid treated West Texas heater oil distillate.<sup>4</sup> Heated for one hour at 200° F. and observed.

The introduction of the additive of the present invention to distillate fuels and the like is greatly facilitated by the use of concentrated oil solutions of such additives. It has, for example, been found especially desirable to use a 10% concentrate of such additive in an oil such as light catalytic cycle oil. A typical concentrate comprises 90% solvent and 10% of an additive consisting of 50% neutralized phosphorus sulfide-hydrocarbon reaction product, 40% alkylene polyamine and 10% carboxylic acid salt of such amine. Such concentrate is used for blending with the oil in whatever proportions may be desired and particularly to obtain a finished product containing the specified percentages of individual constituents. Whereas a 10% concentrate is specifically referred to, it should be understood that such concentration may vary widely and that those as high as 50% or more may be found useful under certain circumstances and are within the scope of the present invention. Moreover, although the light catalytic cycle oil is especially well adapted for use as the carrier or solvent in such a concentrate, any other suitable hydrocarbon oil may be employed.

Percentages given herein and in the appended claims are by weight unless otherwise specified.

Because of the dispersion of water into the oil effected by the additives of the present invention, it is sometimes desirable to employ a surface active agent in addition thereto to prevent hazy oils. Thus, various oil-soluble anionic and cationic surfactants such as the di-alkyl sodium sulfosuccinates, sodium cetyl sulfate, petroleum sulfonates, cetyl pyridinium chloride, octadecylamine acetate, etc. may be employed. Such surfactants will vary in effectiveness with the particular oil, the amount of water, the physical state of the water in the oil, i.e. whether it is suspended, dissolved, etc., the range of temperature over which the oil may be stored, etc., but in general are effective in amounts between about 0.001 to about 0.05% by volume based on total oil. Greater and lesser amounts may be found useful under certain circumstances. Thus, haze was successfully inhibited in a fuel oil composition comprising an oil consisting of 60% virgin furnace oil distillate and 40% catalytic cycle oil which had been stabilized against color and sediment formation with 0.01% of an additive comprising 0.005% of neutralized P<sub>2</sub>S<sub>5</sub> butylene polymer reaction product, 0.004% of Duomeen T and 0.001% of Duomeen T-monooleate, by the addition of 0.002% by volume of sodium mahogany soap derived from the fuming sulfuric acid treatment of a hydrocarbon oil in the preparation of a Technical White Oil. In place of the sodium mahogany soap of the above example, other surfactants of the type above enumerated may likewise be employed.

Having thus described the present invention, what I

claim as novel and desire to protect by Letters Patent is set forth in the following claims.

I claim:

1. A distillate petroleum fuel heavier than gasoline containing from about 0.001% to about 0.1% of a reaction product of a phosphorus sulfide and a non-gaseous higher hydrocarbon which has been neutralized with a basic reagent and from about 0.001% to about 0.1% of an N-alkyl propylene diamine which has the general formula  $\text{RNHCH}_2\text{CH}_2\text{CH}_2\text{NH}_2$  and which contains from about 6 to about 30 carbon atoms in the N-alkyl radical.

2. The composition of claim 1 wherein the N-alkyl group is derived from the alkyl radical of tallow fatty acids.

3. The composition of claim 1 wherein the neutralized reaction product is a reaction product of  $\text{P}_2\text{S}_5$  and an olefin polymer.

4. The composition of claim 1 wherein the neutralized reaction product is a reaction product of  $\text{P}_2\text{S}_5$  and an olefin polymer which has been neutralized with an alkali metal hydroxide.

5. The composition of claim 1 wherein the distillate petroleum fuel is a blend of virgin stocks.

6. A distillate petroleum fuel heavier than gasoline containing from about 0.001% to about 0.1% of a reaction product of a phosphorus sulfide and a non-gaseous higher hydrocarbon which has been neutralized with a basic reagent, from about 0.001% to about 0.1% of an N-alkyl propylene diamine which has the general formula  $\text{RNHCH}_2\text{CH}_2\text{CH}_2\text{NH}_2$  and which contains from about 6 to about 30 carbon atoms in the N-alkyl radical and from about 0.001% to about 0.1% of a higher aliphatic carboxylic acid salt of such an N-alkyl propylene diamine.

7. The composition of claim 6 in which the carboxylic acid is oleic acid.

8. The composition of claim 6 in which the N-alkyl radical is derived from the alkyl radical of tallow fatty acids.

9. The composition of claim 6 in which the reaction product is a reaction product of  $\text{P}_2\text{S}_5$  and an olefin polymer.

10. The composition of claim 9 in which the reaction product has been neutralized with a basic barium compound.

11. The composition of claim 9 in which the reaction product has been neutralized with an alkali metal hydroxide.

12. The composition of claim 11 in which the alkali metal hydroxide is potassium hydroxide.

13. A distillate petroleum fuel heavier than gasoline containing from about 0.001% to about 0.1% of a potassium hydroxide neutralized reaction product of  $\text{P}_2\text{S}_5$  and a butylene polymer, from about 0.001% to about 0.1% of an N-alkyl propylene diamine which has the general formula  $\text{RNHCH}_2\text{CH}_2\text{CH}_2\text{NH}_2$  wherein the N-alkyl radical is derived from the alkyl radical of tallow fatty acids and from about 0.001% to about 0.1% of an oleic acid salt of said N-alkyl propylene diamine.

14. A concentrated solution in a distillate petroleum fraction heavier than gasoline of from about 10 to about 50% of a distillate fuel oil additive comprising about 50% of a reaction product of a phosphorous sulfide and a non-gaseous higher hydrocarbon which has been neutralized with a basic reagent, about 40% of an N-alkyl propylene diamine which has the general formula  $\text{RNHCH}_2\text{CH}_2\text{CH}_2\text{NH}_2$  and which contains from about 6 to about 30 carbon atoms in the N-alkyl radical and about 10% of a higher aliphatic carboxylic acid salt of such an N-alkyl propylene diamine.

30 References Cited in the file of this patent

UNITED STATES PATENTS

|           |               |                |
|-----------|---------------|----------------|
| 2,305,674 | Chenicek      | Dec. 22, 1942  |
| 2,316,080 | Loane et al.  | Apr. 6, 1943   |
| 2,316,087 | Gaynor et al. | Apr. 6, 1943   |
| 2,329,251 | Chenicek      | Sept. 14, 1943 |
| 2,369,490 | Proell        | Feb. 13, 1945  |
| 2,507,731 | Mixon         | May 16, 1950   |
| 2,534,217 | Bartleson     | Dec. 19, 1950  |
| 2,684,292 | Caron et al.  | July 20, 1954  |
| 2,712,528 | Hill et al.   | July 5, 1955   |
| 2,736,658 | Pfohl et al.  | Feb. 23, 1956  |
| 2,771,348 | Meguerian     | Nov. 20, 1956  |